

## UNITED STATES PATENT OFFICE

2,633,471

## WAX MODIFYING AGENT

Eugene Lieber, Chicago, Ill., and Aloysius F. Cashman, Staten Island, N. Y., assignors to Standard Oil Development Company, a corporation of Delaware

No Drawing. Application December 1, 1949,  
Serial No. 130,606

2 Claims. (Cl. 260—407)

1

The present invention relates to the art of producing wax modifying agents particularly those which may be employed for reducing the pour point or waxy lubricating oils or in connection with processes for dewaxing oils containing paraffinic wax or in any other process or composition in which a wax structure is to be modified by reducing the crystal size. The invention will be fully understood from the following description.

In U. S. Patent 2,251,550, granted to E. Lieber, there was described a process of producing an effective wax modifying agent by heat condensation-polymerization of an acid chloride which had been derived from fatty acids containing 10 to 20 carbon atoms. The production of such a material required a step of converting the fatty acid into a fatty acid chloride prior to the heat treatment.

It has now been found, in accordance with the present invention, that satisfactory wax modifying agents may be prepared by the direct pyrolysis of fatty acids and the like. For this purpose, aliphatic carboxylic acids containing 10 to 30 carbon atoms per molecule, the range of 12 to 22 carbon atoms being more generally preferred, are heated at a temperature of 400° F. to 800° F., preferably 500° F. to 700° F., for a period of 1 to 20 hours, more commonly from 4 to 10 hours. While normal atmospheric pressure may be used, reduced pressures are often advantageous in carrying out this process. It is generally advantageous to conduct the heat treatment in the presence of a heat conducting material of large surface area such as steel wool, although such material is not required. The resulting product may be refined in various ways, such as by filtration or distillation to remove raw materials and low boiling condensation products, or by solvent extraction, clay treating, etc.

The exact nature of the chemical process involved is not known, but it is believed that the process is primarily a dehydration-condensation reaction.

The aliphatic acids employed in the process of the present invention may be straight or branched chain compounds, saturated or unsaturated, and may be monobasic or polybasic. Examples of the more preferred acids include stearic acid, palmitic acid, margaric acid, lauric acid, oleic acid, sebatic acid, coconut oil acids, wax oxidation acids, and the like.

The hydrocarbon base stocks into which the wax modifying agents of the present invention are incorporated are preferably waxy mineral

lubricating oils such as a paraffinic lubricating oil base stock or a mixed base, which may have been subjected to any one or more of the commonly used refining steps, such as distillation, solvent extraction, acid treating, clay treating, etc., as well as partial dewaxing. Such oil base stock may either be one which is within the known lubricating oil viscosity range or it may be an oil of much lower viscosity, such as a gas oil used in the preparation of hydraulic oils, etc., and which may have a viscosity as low as 40 seconds Saybolt at 100° F. Solid hydrocarbon base stocks may be used, such as paraffin wax for hot melt coating of paper.

15 In carrying out the invention it is desirable to use the wax modifying additive in proportions of about 0.1 to 5% based on the lubricating oil base stock, although usually 1% is sufficient for most purposes. It will be understood that different oils require slightly different amounts of the material to produce a given drop in pour point, and likewise material prepared from different types of acids vary somewhat in their pour depressing strength.

20 The wax modifying agents of the present invention may be used in connection with the process for dewaxing hydrocarbon oils and then added either to the oil to be dewaxed or to the oil after it has been diluted with naphtha or with other suitable dewaxing solvents. The mixture is chilled to the wax separating point and the actual separation may be conducted either by filtration, sedimentation or centrifugation. In any case it will be found that the presence of

25 a relatively small amount of the material, say 1% more or less, will considerably increase the ease with which the separation is accomplished and increase the rate at which chilling may be carried out.

30 The desirable results obtained by the use of the additives described in the present specification may be illustrated by the following example which, however, is not to be considered as limiting the scope of the invention in any way.

35

40

45

*Example*

400 g. of commercial stearic acid and 10 g. of steel wool were placed in a Claisen flask and heated at 600° F. for 6 hours. The product was 45 recovered by vacuum distillation to 600° F. under a pressure of 75 mm. mercury. The steel wool was removed from the product by filtering the bottoms from the distillation step through a steam funnel. A yield of 247 g. of a dark waxy material 50 was obtained. The pour depressing potency of

this product was tested by blending 1% by weight of the same in a waxy base oil consisting of 80 parts by weight of a light paraffinic lubricating oil of the white Pennsylvania type and 20 parts of Pennsylvania bright stock, the blend having a viscosity of 50 seconds Saybolt at 210° F. The unblended base stock exhibited a pour point of +30° F. as determined by the standard ASTM procedure while the blend containing 1% of the additive exhibited a pour point under this procedure of -30° F.

This application is a continuation-in-part of Serial No. 789,576, filed December 3, 1947, for the same inventors which is now abandoned.

What is claimed is:

1. A process for the formation of a material having the characteristic of lowering the pour point of waxy mineral oils which comprises heating stearic acid at a temperature of from 500° F.

to 700° F. for a period of from 4 to 10 hours in the presence of steel wool.

2. A process according to claim 1 wherein the temperature is about 600° F. and the time of heating is about 6 hours.

EUGENE LIEBER.  
ALOYSIUS F. CASHMAN.

#### REFERENCES CITED

10 The following references are of record in the file of this patent:

#### UNITED STATES PATENTS

|    | Number    | Name            | Date           |
|----|-----------|-----------------|----------------|
| 15 | 2,201,767 | Franceway       | May 21, 1940   |
|    | 2,256,353 | Rheineck et al. | Sept. 16, 1941 |
|    | 2,349,165 | Grant           | May 16, 1944   |
|    | 2,373,015 | Cowan et al.    | Apr. 3, 1945   |